

No. 645,205.

Patented Mar. 13, 1900.

F. W. HAWKINS.

PROCESS OF REFINING IRON.

(Application filed May 6, 1899.)

(No Model.)

Fig. 1.



Fig. 2.



Witnesses  
J. C. Smith  
McDougherty

Investor  
F. W. Hawkins  
By Thos. Sprague, Atty.

# UNITED STATES PATENT OFFICE.

FREDERICK W. HAWKINS, OF DETROIT, MICHIGAN, ASSIGNOR OF ONE-FIFTH  
TO THOMAS A. E. WEADOCK, TRUSTEE, OF SAME PLACE.

## PROCESS OF REFINING IRON.

SPECIFICATION forming part of Letters Patent No. 645,205, dated March 13, 1900.

Application filed May 6, 1899. Serial No. 715,859. (No specimens.)

*To all whom it may concern:*

Be it known that I, FREDERICK W. HAWKINS, a citizen of the United States, residing at Detroit, in the county of Wayne and State 5 of Michigan, have invented certain new and useful Improvements in Processes of Refining Iron, of which the following is a specification, reference being had therein to the accompanying drawings.

10 The invention relates to a method of refining metal, and has particular reference to the refining of iron for the manufacture of steel.

It is the object of the invention to more quickly and thoroughly eliminate from the 15 metal certain impurities of detrimental character, such as phosphorus, which do not readily yield to processes of oxidation, as in the Bessemer converter.

To this end my invention consists in the 20 method hereinafter described and claimed.

In the drawings I have shown in diagram an apparatus capable of carrying out my improved method, and in which—

25 Figure 1 is a diagram longitudinal section, and Fig. 2 a horizontal section.

My improved method consists, essentially, in two steps, which, however, are preferably carried out without interruption in a single apparatus. The first of these steps consists 30 in the atomizing or breaking up of the molten metal into minute particles. This is accomplished by subjecting a thin stream of the metal to the action of a strong blast, which is directed laterally against the stream and preferably inclined slightly upward, so as to break 35 up the metal and scatter the particles.

In the drawings I have shown an open-hearth furnace A, projecting into one end of which is a steam-pipe B, terminating in a 40 nozzle C, this nozzle being located, preferably, above one end of the hearth.

D is an inlet for the molten metal, which is formed by a narrow slit in the roof of the furnace.

45 E is an air-twyer arranged above the steam-inlet C and preferably inclined slightly downward. With this arrangement the molten

metal falling in a thin stream through the inlet D will pass directly in front of a steam-nozzle C, through which a powerful blast of steam, preferably superheated, is directed laterally against the stream and breaks it up in the manner above described, scattering the particles over the entire length of the hearth, upon which they will fall in the form of a fine 55 rain. At the same time air, preferably pre-heated, enters through the twyer E and is directed against the stream of molten metal above the steam-jet and assists in atomizing the metal. The effect of this combined action 60 of air and steam on the molten metal is, in addition of the mechanical result of atomizing the same, also to produce a strong oxidizing influence upon the particles during their passage through the furnace. 65

The second step of my method consists in filtering divided particles of metal through a bed of crushed or comminuted basic material. This material is strewn over the hearth, as shown at F, of the furnace and is heated to a 70 high temperature before the metal is introduced into the furnace. Thus when the particles of molten metal drop upon this basic bed they will be compelled to filter through the same and in so doing will be brought into 75 such intimate relation with the basic as to thoroughly eliminate the phosphorus and other impurities of like nature. As the metal collects at G below the basic bed the latter will be raised, so that the action will continue 80 until the entire charge of metal has been thus atomized and filtered through.

It will be readily understood that this method of treatment can only result in a homogeneous mass of purified iron, as every 85 particle is subjected to precisely the same chemical influences, whereas in other processes where the metal is treated in bulk no such uniformity in result can be obtained. Furthermore, by my process the time required 90 for the purification of the iron is greatly diminished over other processes in which the metal is treated in the open-hearth furnace.

I claim—

1. A method of refining iron consisting in first atomizing or breaking up into minute particles and scattering of the molten metal, and in then filtering the separate particles through a bed of comminuted basic material.

2. The herein-described method of refining iron consisting in first atomizing or breaking up and scattering the molten metal into minute particles by a blast and in then filtering

the separate particles through a heated bed of comminuted basic material.

In testimony whereof I affix my signature in presence of two witnesses.

FREDERICK W. HAWKINS.

Witnesses:

JAMES WHITTEMORE,  
M. B. O'DOGHERTY.